

Feb. 24, 1925.

1,527,293

W. T. BONNER

FRICITION MEMBER

Filed March 18, 1920



Fig. 2.



Inventor:  
William T. Bonner,  
By Clyde L. Roque  
his Atty.

Patented Feb. 24, 1925.

1,527,293

# UNITED STATES PATENT OFFICE.

WILLIAM T. BONNER, OF TRENTON, NEW JERSEY, ASSIGNOR TO MAX BROWN, OF BOSTON, MASSACHUSETTS.

## FRICITION MEMBER.

Application filed March 18, 1920. Serial No. 366,944.

To all whom it may concern:

Be it known that I, WILLIAM T. BONNER, a citizen of the United States, residing at Trenton, in the county of Mercer and State 5 of New Jersey, have invented a new and useful Improvement in Friction Members, of which the following is a specification.

I have discovered that the alkaline metal magnesium, and alloys thereof hereinafter 10 described, possess friction value of a high order and sufficient strength to transmit power. I have also discovered that the coefficient of friction of magnesium and its alloys may be increased by alloying there- 15 with either of the metals sodium, potassium, or calcium, and that the tensile strength of a friction member made of such metal or alloys may be increased by alloying manganese therewith. By alloying from two to 20 three parts of the metal manganese with ninety-eight or ninety-seven parts of the metal magnesium I produce an alloy possessing greater tensile strength than is possessed by the pure metal magnesium without 25 an appreciable loss of its friction value. The friction value of such described alloy can be increased, if desired, by the addition of the metal sodium in the proportion of one-half of one part of sodium to ninety- 30 nine and one half parts of the said alloy. The proportions of the different metals in the alloys mentioned may be varied somewhat without seriously changing the mentioned qualities of the alloys, but I prefer 35 to adhere rather closely to the proportions which I have named. Either the metal potassium or the metal calcium may be substituted for the metal sodium in such alloys in similar proportions with similar results.

40 The metal sodium, like potassium or calcium, being of an unstable nature and a rapid absorbent of oxygen, imparts that quality, in a lesser degree, to such alloy of which it is a constituent element and raises 45 the friction value of the alloy.

While I describe and prefer for the uses mentioned, the metal magnesium and its alloys, I have also discovered that other metals, such as aluminum, zinc, and copper, when alloyed with what are known as "unstable metals", such as sodium, potassium, and calcium, obtain a capacity for the absorption of oxygen in a greater degree than is possessed by such metals when unalloyed, resulting in a large gain of friction

value; and this without the loss of that tensile strength which is essential to their use in friction members. The metal magnesium, unalloyed, I have also found to possess a desirable co-efficient of friction and sufficient tensile strength to be useful as a material for friction elements without being used in excessive mass in construction.

The lightness, or low specific gravity, of magnesium, and its described alloys, their 65 high friction value, and their remarkable endurance of frictional wear, make them very desirable as materials for use in the construction of friction members, such as clutches and brakes; and especially so when 70 such friction elements are used in automotive vehicles in which the combined qualities of lightness, strength and durability of parts are highly essential.

Viewed, then, in its broad aspect, my invention consists in the utilization of my discovery of the friction values of the aforesaid metal magnesium and of various alloys, by constructing friction members of said materials, whereby great advantages 80 are gained in reduction of mass, diminution in weight, greater efficiency, and largely increased longevity of such members in service.

In this specification I illustrate my invention as embodied in clutch mechanism of 85 a form in common use in automotive vehicles.

In the clutch or friction drive, as employed chiefly on automotive conveyances, 90 to transmit the power of the engine to the driving mechanism, one or more metal discs are employed. Where only one disc is used the clutch or drive is usually known as a "single disc clutch," while, if a plurality of discs are used, the construction is known 95 as a "multiple disc clutch." The metal heretofore used in the construction of these discs is iron or steel, which is selected solely for its strength, and, as the metal lacks an 100 adequate co-efficient of friction to transmit the power received by the discs to such contacting surfaces as they are intended to engage, it has been necessary to face the discs with a material having a friction value 105 exceeding that of the metal discs. The material used for this purpose is commonly composed of a fibrous substance or a fabric, united and hardened by a cementitious binder. In the construction of single disc 110

clutches the disc is frequently made wholly of such fibrous or fabric material so united and hardened. The friction discs described, when composed of a metal disc with a facing 5 of fibrous or fabric material on one or on each of its faces, is a composite structure expensive to manufacture and has to be frequently replaced because of the wear and destruction of its frictional facings, while 10 the discs made wholly of fibrous or fabric material are subject to the same objections. By constructing these friction discs of a metal or alloy possessing both the requisite tensile strength and a high friction value 15 I reduce the bulk of those elements, the size of their housings, and the weight of the entire structure of the clutch, and obtain a greatly increased length of service, approximately equal to that of the other 20 parts of the mechanism with which they are combined, while the cost of the original construction is materially lessened.

Referring to the drawings forming a part 25 of this specification, wherein an illustrative embodiment of the invention is shown,

Fig. 1 shows in side elevation a clutch element embodying the invention;

Fig. 2 is a transverse diametrical section thereof;

Fig. 3 is an elevation showing a preferred 30 form of clutch disc with attached friction-facing in common use; and,

Fig. 4 is a transverse diametrical section thereof.

10 indicates a clutch disc which may be employed for either a multiple disc clutch or a single disc clutch. This disc is composed of metallic magnesium, or a suitable alloy thereof, or, in a broader aspect, it may 15 be composed of other materials, already named as having a relatively high co-efficient of friction, while also having sufficient inherent strength and toughness to withstand the service usage in a clutch without other 20 reinforcement or backing. This disc or ring may be equipped with notches or projections for engaging a key-way in its periphery, as indicated at 10<sup>a</sup>. It will be understood that 25 these notches or key-way engagements are produced upon the outer periphery of the ring, since these rings or discs correspond to, and are to take the place of the composite discs equipped with friction rings or facings hitherto employed. The intermediate 30 metal discs, usually of iron or steel, operate directly against the faces thereof, having their engaging notches or key-ways upon the inner circle or periphery of the ring. This improved friction element thus 35 takes the place of the composite ring illustrated in Figs. 3 and 4, wherein a metallic packing ring 11 of iron or steel and

equipped with outer peripheral notches, 11<sup>a</sup> is provided, and on one or both sides thereof friction facings, 12, are secured by riveting, or otherwise. These faces are usually of a composition comprising compressed fibrous or textile material united with a suitable cementitious binder.

As other modifications and specific forms 70 of the invention may be employed, I desire the present embodiment to be considered in all respects as illustrative, and not restrictive, and refer to the appended claims rather than to the foregoing description, to indicate the scope of the invention, which, in effect, is the construction of friction members, in the broad sense of that term, of whatever form, or to whatsoever use they may be applied, of the metal, or alloys, 75 80 possessing the friction value referred to herein.

Having described my invention, what I claim as new and desire to secure by Letters Patent, is;

1. A friction member comprising upwards 85 of ninety percent of metallic magnesium, and less than ten percent of an alkaline metal as described, possessing sufficient strength to receive transmitted power and a relatively high co-efficient of friction to deliver the power so received to one or more contacting elements.

2. A friction member of metallic magnesium possessing, as described, sufficient 90 inherent strength to receive upon its surface or periphery, transmitted power, and possessing a relatively high friction value, sufficient to transmit frictionally from its operative sides or faces, the power so received to one or more contacting surfaces.

3. A friction member comprising upwards 95 of ninety percent of metallic magnesium alloyed with a minor proportion of strength giving metal as described, possessing sufficient inherent strength to receive transmitted power, and possessing upon its operative sides or faces a relatively high value 100 in friction efficiency adapted to transmit the power received to one or more contacting 105 surfaces.

4. A friction member for clutches of automotive vehicles, of metallic magnesium in one piece, possessing, as described, sufficient 110 strength to receive upon its surface or periphery power transmitted, and possessing a relatively high friction value sufficient to transmit from its operative sides or faces frictionally, the power so received to one or more contacting surfaces.

In testimony whereof, I have signed my name to this specification.

WILLIAM T. BONNER.